

## UNITED STATES PATENT OFFICE

2,467,334

## FUSE POWDER COMPOSITION

George C. Hale and David Hart, Dover, N. J.

No Drawing. Application July 5, 1944,  
Serial No. 543,580

2 Claims. (Cl. 52—2)

(Granted under the act of March 3, 1883, as  
amended April 30, 1928; 370 O. G. 757)

1

The invention described herein may be manufactured and used by or for the Government for governmental purposes without the payment to us of any royalty thereon.

The present invention relates to the employment of metallic alloys in combination with solid non-metallic elements, to form substantially gasless fuze powder compositions which are intended for use primarily in powder trains of ammunition to provide a definite burning time interval.

The present invention is closely related to an application filed in our names on June 9, 1944, bearing Serial Number 539,504, now Patent No. 2,461,544. In that application we made claim to the use of metals in combination with solid non-metallic elements to form substantially gasless fuze powder compositions.

We have also discovered that in certain particular cases, it is preferable to use a metallic alloy rather than the metal. While the alloys offer little advantage over the metals, with respect to establishing the proper timing in a particular component, or in obtaining uniformity in rate of burning, other advantages have been found from the standpoint of manufacture, storage, and economy. For example, alloys of magnesium are more brittle and hence more readily reduced to finely divided powder than the metal alone. Another advantage in the use of certain alloys resides in the fact that particular alloys may be commercially available while the component parts of the alloys may not be readily procurable. A still further advantage lies in the fact that certain particular metal alloy compositions are more stable than the particular metals making up such alloys.

The invention can best be understood from the following particular exemplifications, which, however, are not to be understood as limiting the scope of the invention and are cited merely as illustrative examples.

| Example |                    | Per-<br>cent |           | Per-<br>cent | Burning<br>Time |
|---------|--------------------|--------------|-----------|--------------|-----------------|
| 1       | Ferrovanadium      | 80           | Sulfur    | 20           | 7               |
| 2       | Manganese-Titanium | 90           | Sulfur    | 10           | 5               |
| 3       | Barium-Silicon     | 95           | Sulfur    | 5            | 11              |
| 4       | Barium-Silicon     | 80           | Tellurium | 20           | 9               |
| 5       | Barium-Silicon     | 90           | Selenium  | 10           | 19              |

2

The burning time indicated in each of the examples above is that of powder column 2" long x 0.22" diameter. While in the examples shown above, we have indicated the use of barium alloys,

- 5 it is to be understood that we do not limit the invention to the particular barium alloys shown, and we envisage the fact that certain other alkaline earth metal alloys can be used to secure results comparable to those set forth.
- 10 Test data also shows that the burning rates of fuze powder compositions containing metal alloys and solid non-metallic elements can be varied over a wide range by varying the proportions of alloy to the solid non-metallic element. These 15 new fuze powder compositions are very readily prepared, but careful control of the particle size of the ingredients is essential. It is desirable that the alloys and non-metals be finely divided so as to pass through a 250 mesh screen. Dry 20 incorporation may be used or the compositions may be mixed with water or any other liquid necessary to avoid accidental ignition in manufacture. After thorough incorporation, the fuze powders are granulated in commercially available 25 mechanical granulators or by passing through screens. Although binding agents have not been found necessary to assist in granulating these powders, one may be used if special cases require it.

Having thus described the invention what is 30 claimed as new is:

1. A substantially gasless delay powder train formed of a mixture of about 90% of finely divided manganese-titanium alloy and about 10% of finely divided sulphur.
- 35 2. A substantially gasless delay powder train formed of a mixture of about 90% of manganese-titanium alloy sufficiently finely divided to pass through a 250 mesh screen and about 10% of sulphur sufficiently finely divided to pass through 40 a 250 mesh screen.

GEORGE C. HALE.  
DAVID HART.

## REFERENCES CITED

45 The following references are of record in the file of this patent:

## UNITED STATES PATENTS

- 50 Number Name Date  
1,971,502 Piccard Aug. 28, 1934  
2,185,371 Burrows et al. Jan. 2, 1940